

Oct. 13, 1959

W. R. KEEN ET AL

2,908,013

COATED TEXTILE MATERIAL AND METHOD OF MAKING SAME

Filed May 9, 1957

FIG. 1.



FIG. 2.



FIG. 3.



FIG. 4. TUFTING MACHINE



FIG. 5.



INVENTORS:  
Edwin Joseph Grajeck and  
William Rollin Keen,  
BY

Paul & Paul  
ATTORNEYS

# United States Patent Office

2,908,013

Patented Oct. 13, 1959

1

2,908,013

## COATED TEXTILE MATERIAL AND METHOD OF MAKING SAME

William Rollin Keen, Media, and Edwin Joseph Grajeck, Malvern, Pa., assignors to Collins & Aikman Corporation, New York, N.Y., a corporation of Delaware

Application May 9, 1957, Serial No. 658,150

3 Claims. (Cl. 2—278)

This invention relates to a new coloring material used in the backing material of a tufted fabric and to a method of making such a fabric. More particularly the invention relates to decoratively coated jute woven backings used in carpets.

Carpets have heretofore been made by tufting textile yarns in a woven jute backing material. Such carpets were dyed with a coloring material to provide an interesting and decorative appearance. However the jute backing material does not accept the dyes normally used and in the resulting carpet there have been noticeable differences in shade between the pile tufts and the backing material. Since the backing material in a tufted fabric is normally somewhat visible through the pile this discrepancy in coloring detracts from the appearance of the fabric.

It has also been a problem in the manufacture of tufted fabrics and particularly carpet materials that the meshes in the backing material are not regular and uniform. Due to this the tufting needles have often distorted the original strand alignments of the backing material during the tufting operation thereby disrupting the normal surface of the backing material with an attendant loss of uniformity in the resulting product.

It is a principal purpose of this invention to provide a decorative, colored coating material to be applied to the upper surface of the woven jute backing material for a tufted carpet which will harmonize in color with the tufted pile yarns and will in addition provide stability to the backing material during the tufting operation.

It is also an object of this invention to provide a colored coated backing material for tufted carpets which will harmonize in color with the yarns tufted in said backing material and which will essentially resist the distorting stresses occasioned by the passage of tufting needles through the backing material.

2

It is another object of this invention to provide a tufted carpet having a jute woven backing coated with a latex material adapted to retain coloring matter which will harmonize with the color of the pile tufts of said carpet and which will enhance the stability of the backing material of the carpet.

It is still another object of this invention to provide a method of making a tufted carpet in which a latex coating material is applied to the backing of the carpet prior to tufting so that the backing material will not be distorted by the passage of tufting needles.

Other objects and advantages of the invention will become apparent from the following description and the drawings of which:

Fig. 1 is a perspective view of a piece of jute backing material of the type normally used in the manufacture of tufted carpets;

Fig. 2 is a schematic view showing an application of the colored coating material to the backing material of Fig. 1 in accordance with the invention;

Fig. 3 is an enlarged, partial, side elevation of the backing material of Fig. 1 following the treatment of Fig. 2;

Fig. 4 is a schematic view showing the tufting and shearing of the backing material following the treatment of Fig. 2; and

Fig. 5 is a partial perspective view of the tufted material following the operation of Fig. 4.

The backing material 10 illustrated in Fig. 1 is typical of the backing material presently used in the manufacture of tufted carpets. It will be noted that the woven fabric 10 is not regular and uniform and that there are substantial variations in the alignment of the weft strands 11 and the warp strands 12 and the positioning of the meshes.

It has been found that when such a backing material is tufted to form a carpet in the normal manner two problems arise. The tufting operation results in distortion of the backing material 10 due to the tufting needles striking the strands 11 and 12 in different places, and after the backing material 10 is tufted and is dyed to provide color the jute backing material does not accept the dye to produce the same shade as the normal textile material used in the pile yarns. It has been determined that both of these problems may be largely solved by coating the fabric 10, prior to tufting, with a latex material carrying the desired coloring material in solutions or dispersions. Specific examples of particular compositions which have

been found satisfactory for this are listed below:

### EXAMPLE #1

| Chemical Classification            | Commercial Product   | Vendor      | Formula in Pounds |
|------------------------------------|----------------------|-------------|-------------------|
| Acrylic resin dispersion           | Rhoplex AC-33        | Rohm & Haas | 100               |
| Sodium polyacrylate thickener (5%) | Acrysol GS           | Rohm & Haas | 10                |
| Phthalocyanine Blue Paste          | Monastral F. Blue BC | Du Pont     | 5                 |

### EXAMPLE #2

|                                |                      |             |     |
|--------------------------------|----------------------|-------------|-----|
| Acrylic resin dispersion       | Rhoplex AC-33        | Rohm & Haas | 100 |
| Sodium alginate thickener (3%) | Keltex               | Kelco Co.   | 50  |
| Phthalocyanine Blue Paste      | Monastral F. Blue BC | Du Pont     | 5   |

### EXAMPLE #3

|                                |                      |                         |     |
|--------------------------------|----------------------|-------------------------|-----|
| Compounded GRS-Rubber Latex    | Vulcanol 2009        | Alco Oil & Chemical Co. | 100 |
| Sodium alginate thickener (3%) | Keltex               | Kelco Co.               | 30  |
| Phthalocyanine Blue Paste      | Monastral F. Blue BC | Du Pont                 | 5   |

## EXAMPLE #4

| Chemical Classification                              | Commercial Product             | Vendor                 | Formula in Pounds |
|------------------------------------------------------|--------------------------------|------------------------|-------------------|
| Acrylonitrile Polymer Dispersion                     | Nitrex 2614                    | Naugatuck Chemical Co. | 100               |
| Sodium alginate thickener (3%)                       | Keltex                         | Kelco Co.              | 50                |
| Vat Dye Color Index #1101 (Dimethoxy Dibenzanthrone) | Ponsol Jade Green Double Paste | Du Pont                | 10                |

## EXAMPLE #5

|                                                      |                                |                         |                  |
|------------------------------------------------------|--------------------------------|-------------------------|------------------|
| Compounded GRS-Rubber Latex                          | Vulcanol 2009                  | Alco Oil & Chemical Co. | 39 $\frac{1}{4}$ |
| Acrylonitrile Polymer Dispersion                     | Nitrex 2614                    | Naugatuck Chemical Co.  | 66 $\frac{2}{3}$ |
| Sodium alginate thickener (3%)                       | Keltex                         | Kelco Co.               | 43 $\frac{1}{3}$ |
| Phthalocyanine Blue Paste                            | Monastral F. Blue BG           | Du Pont                 | 1 $\frac{1}{3}$  |
| Vat Dye Color Index #1101 (Dimethoxy Dibenzanthrone) | Ponsol Jade Green Double Paste | Du Pont                 | 6 $\frac{2}{3}$  |

In addition to the above, copolymers of vinyl chloride and vinyl acetate may be used in place of acrylic acrylonitrile, or rubber binders. Compatible mixtures of these binders are also satisfactory. In any event the binder material should not be less than equal in amount to the pigment used and can be present in any amount above that, which will still give a good spreading dispersion. While sodium alginate is set forth as the thickener in these examples any thickener such as carob gum, methyl cellulose and the like which are compatible with the dispersion may be used. Of course, any desirable pigment may be used.

The coating material 13 may be applied to the backing material 10 in any known manner for applying coatings to fabrics. For example, as shown in Fig. 2 the coating 13 may be applied by means of rollers 14, 15 and 16 drawing the material 13 from container 17. It will be noted that it is only necessary to apply the coating 13 to one side of the backing material 10.

When the backing material 10 has been coated the coating material 13 is distributed across the upper surface of the yarns 11 and 12 without substantial filming between parallel strands, but "cementing" the yarns at the cross-overs. It is, of course, desirable to maintain the meshes of the fabric 10 open as far as possible to avoid placing any additional strain on the tufting needles and the tufting machine.

The coated backing material 10 is then fed in the usual manner through a tufting machine 18 in which the pile yarns 19 are tufted into backing material 10. Where a sheared pile fabric is desired the loops of the yarns 19 are cut by means of shearing knife 20.

The resulting product shown in Fig. 5 is a tufted pile fabric in which the backing material is provided with a coloring which harmonizes with the coloring of the pile yarns after the pile yarns have been dyed. The pile yarns are dyed the desired color in the usual manner subsequent to shearing. It will be noted, as shown in Fig. 5, that, due to the tufting operation, strands 11 and 12 of backing material 10 and particularly weft strands 11 are distorted in position by the tufting operation. The application of the coated material 13 provides great stability in the backing material 10 tending to resist distortion. The resulting fabric has much greater fabric stability.

As is customary in the art of tufted carpets a binding composition is applied to the back of the backing material

10 to insure the retention of the tufted pile yarns 19 in the backing material 10. Such a binding material is indicated at 21 in Fig. 5.

20 It will be understood that numerous variations may be made in the steps and elements of the invention without departing from the scope thereof as defined by the following claims.

25 Having thus described our invention, we claim:

1. A tufted pile fabric comprising a woven backing material, a plurality of colored textile yarns tufted in said backing material, having a specific color producing a specific visual color effect a first colored coating material applied to the upper surface of said backing material having a pigment contained therein producing the same visual color effect as the color in said pile yarns and a second coating material applied to the under side of said backing material to retain said pile yarns in place in said backing material.

30 2. A method of making a tufted pile carpet comprising the steps of first coating a woven jute backing material on one side with a dispersion of a specific coloring pigment in latex, then tufting a plurality of textile yarns in said backing material, then dyeing said tufted yarns with a dye having a pigment producing the same visual color effect as the pigment of the dye applied to said backing material and then coating the backing material on the side opposite said first coating with a binder material to 35 retain the pile yarns in place.

3. A method of making a tufted pile carpet having tufted yarns dyed with a specific coloring pigment comprising the steps of first coating a woven jute backing material on one side with a dispersion in latex of a coloring pigment producing the same visual color effect as the pigment in the dye of said tufted yarns, then tufting a plurality of said textile yarns dyed with said specific coloring pigment in said backing material and then coating the backing material on the side opposite said first coating with a binder material to retain the pile yarns in place.

## References Cited in the file of this patent

## UNITED STATES PATENTS

|    |           |           |               |
|----|-----------|-----------|---------------|
| 60 | 2,042,503 | Carter    | June 2, 1936  |
|    | 2,220,589 | Unger     | Nov. 5, 1940  |
|    | 2,261,096 | Reinhardt | Oct. 28, 1941 |
|    | 2,314,162 | Reinhardt | Mar. 16, 1943 |
|    | 2,630,620 | Rand      | Mar. 10, 1953 |

UNITED STATES PATENT OFFICE  
CERTIFICATE OF CORRECTION

Patent No. 2,908,013

October 13, 1959

William Rollin Keen et al

It is hereby certified that error appears in the printed specification of the above numbered patent requiring correction and that the said Letters Patent should read as corrected below.

Column 1, line 34, for "Dus" read — Due —.

Signed and sealed this 19th day of April 1960.

(SEAL)  
Attest:

KARL H. AXLINE  
Attesting Officer

ROBERT C. WATSON  
Commissioner of Patents